

# UNITED STATES PATENT OFFICE.

ANTON TYPLT, OF MUNICH, GERMANY.

## PROCESS OF MAKING PAVING-STONES.

SPECIFICATION forming part of Letters Patent No. 532,118, dated January 8, 1895.

Application filed September 18, 1893. Serial No. 485,409. (No specimens.) Patented in England July 4, 1893, No. 13,079; in Belgium July 11, 1893, No. 105,515; in Italy August 8, 1893, No. 34,613, and in Switzerland September 13, 1893, No. 7,568.

*To all whom it may concern:*

Be it known that I, ANTON TYPLT, a subject of the King of Bavaria, and a resident of Munich, Bavaria, in the German Empire, have 5 invented a certain new and useful Improved Process for Making Paving-Stones, Patterned Slabs, and the Like, (for which I have obtained the following patents: in Switzerland, No. 7,568, dated September 13, 1893; in Belgium, No. 105,515, dated July 11, 1893; in England, No. 13,079, dated July 4, 1893, and in Italy, No. 34,613, dated August 8, 1893,) of which the following is a full, clear, and exact description.

15 The object of the present invention is to produce paving stones or slabs, as also patterned slabs and the like, from waste granite, syenite and basalt.

In order to obtain this object eight or nine 20 parts by weight of waste of one or the other of the above mentioned stones—according to the color or the kind of slab required to be produced—are added to one hundred parts by weight of magnesia and worked up with 25 a solution of chloride of magnesium, the latter of a consistency of 25° to 30° Baumé, to a thick pulpy mass. The mixture thus obtained is then cast into rigid mold,—for instance cast iron molds—and allowed to harden which 30 takes place in about seventy-eight hours.

It is absolutely necessary that the molds into which the mixture is cast be of a rigid unyielding nature, in order to obtain perfectly hard infrangible slabs, the rigid mold preventing the expansion of the mass and consequently compressing and rendering the same more compact. 35

If it is required to produce patterned or designed slabs the coloring matters employed must be of such a nature that the same will 40 easily dissolve in the chloride of magnesium solution and without changing or losing their color.

I claim as my invention—

A process for producing paving and de- 45 signed slabs and the like, consisting in mixing eight to nine parts of the waste of basalt, syenite or granite stone with one hundred parts of magnesia and working the same up with a solution of chloride of magnesium to 50 a thick or pulpy mass and then casting the mass thus obtained into rigid molds, and allowing it to harden there, substantially as described.

In witness whereof I hereunto set my hand 55 in presence of two witnesses.

ANTON TYPLT.

Witnesses:

W. BANTZE,  
H. SCHLOSS.